

# UNITED STATES PATENT OFFICE.

JESSE L. JONES, OF OAKMONT, PENNSYLVANIA, ASSIGNEE TO WESTINGHOUSE ELECTRIC AND MANUFACTURING COMPANY, A CORPORATION OF PENNSYLVANIA.

## METHOD OF ETCHING METALS.

1,248,499.

Specification of Letters Patent.

Patented Dec. 4, 1917.

No Drawing.

Application filed June 11, 1915. Serial No. 33,510.

*To all whom it may concern:*

Be it known that I, JESSE L. JONES, a citizen of the United States, and a resident of Oakmont, in the county of Allegheny and State of Pennsylvania, have invented a new and useful Improvement in Methods of Etching Metals, of which the following is a specification.

My invention relates to methods of testing the physical properties of metals, and it has special reference to methods of etching iron, steel and other industrial metals for the purpose of microscopic examination.

The object of my invention is to provide a method of etching metals by means of which irregularities in composition and structure may be made evident in a simple and convenient manner.

The microscopic examination of metals by polishing the surface of small samples and then etching with various reagents has been brought to a high degree of excellence, especially in the iron and steel industries. Less progress has been made, however, in the development of methods of rendering visible on a large scale the porosity, irregularity in composition, hair cracks, blisters, seams and other defects which are difficult to detect by visual inspection in rolled or forged metals, where the mechanical working has rendered the surface of the metal apparently uniform.

I have discovered that iron, steel and other metals may be etched to a marked degree by immersing them for a short time in a molten metal of lower melting point. For the treatment of iron and steel, I prefer to use molten zinc as the etching reagent, but other metals of relatively low melting point such as molten tin, lead and hot mercury may also be used.

In etching metals according to my method, samples of the metals to be tested are suspended for one or more hours in a bath of molten zinc maintained at a uniform temperature. I have found it desirable to provide a mechanical arrangement that will keep the articles being etched in constant motion while in the molten zinc. Five hours is a suitable immersion period for producing thorough etching. The samples are then taken from the molten zinc, the adherent dross and metallic zinc are broken off as much as possible by means of a hammer, and the samples are finally cleaned by immersing

in dilute sulfuric acid, which does not attack the metal of the samples as long as any zinc remains. Metals treated in the foregoing manner are found to be etched in such a manner as to indicate very plainly the homogeneity and surface condition of the metal.

The action of molten zinc upon steel and iron appears to be in direct proportion to the amount of carbon present at the surface of the test samples, the zinc dissolving steel that is high in carbon much more readily than carbon-free iron. This fact renders it possible to determine accurately the uniformity of carbon steel, since the areas high in carbon are deeply eroded. Case-hardened iron and steel can also be tested by this method to show the depth and character of the surface hardening. Porous areas are also attacked by the molten zinc, being much more readily dissolved than non-porous areas, which in comparison are scarcely attacked at all.

Another application of the foregoing method is in the examination of high-speed steels containing additions of tungsten, chromium, manganese, vanadium, cobalt, etc. These steels are etched in a very irregular manner which indicates that the constituent metals are seldom, if ever, perfectly alloyed. The deeply etched spots in such steels are probably very high carbon areas that are vigorously attacked by the molten zinc.

While I have specifically described the treatment of iron and steel samples with molten zinc, it is to be understood that my invention is not restricted to the examination of iron and steel or to the use of zinc as the etching reagent. The use of molten lead for etching platinum and platinum-iridium alloys has been found advantageous. Any metal or mixture of metals may be used as the etching reagent which is molten at a lower temperature than the metal to be etched, and it is therefore to be understood that my invention comprises all modifications in materials and methods that fall within the scope of the appended claims.

I claim as my invention:

1. The method of etching metals that comprises immersing the metal to be etched in a molten metal of lower melting point that is capable of alloying with the metal to be etched, removing the etched metal from the molten bath, breaking off the adherent ma-

60

65

70

75

80

85

90

95

100

105

110

terial, and treating the etched metal with a solvent of the reagent metal.

2. The method of etching metals capable of alloying with zinc that comprises immersing the metal to be etched in molten zinc, removing the etched metal from the molten bath, breaking off the adherent material, and treating the etched metal with dilute sulfuric acid.

10 3. The method of etching metals that

comprises immersing the metal to be etched in a molten metal of lower melting point that is capable of alloying with the metal to be etched, agitating the said molten metal, removing the etched metal from the molten 15 bath, and cleansing the said etched metal.

In testimony whereof, I have hereunto subscribed my name this 27th day of May, 1915.

JESSE L. JONES.